

## UNITED STATES PATENT OFFICE

2,046,629

## PROCESS OF CEMENTATION

Harry K. Ihrig, Milwaukee, Wis., assignor to  
Globe Steel Tubes Co., Milwaukee, Wis., a cor-  
poration of Delaware

No Drawing. Application June 25, 1934,  
Serial No. 732,305

13 Claims. (Cl. 91—70.1)

This invention relates to the coating and im-  
pregnating of metals, particularly iron and steel,  
with other metals by a process of cementation.

It has heretofore been proposed to coat a  
5 metal by processes of cementation wherein the  
metal to be coated is heated in contact with the  
coating metal in powdered form. Under these  
prior proposals, however, extremely anhydrous  
conditions, high temperatures, and special pro-  
10 visions for rigid reducing atmospheres were  
necessary as well as long periods of heating.  
Other objections and disadvantages were also  
inherent in these prior processes which, coupled  
with the negligible degree of penetration of the  
15 coating metal into the grain structure of the  
foundation metal, rendered such practices as  
well as the resultant products of little or no  
practical or commercial value.

According to the present invention, coating and  
20 impregnation are obtained at relatively low  
temperatures and with no necessity for the main-  
tenance of the extreme conditions above out-  
lined. Furthermore, the results are superior in  
that the depth of the coating and impregnation  
25 or case is substantial and of such character as  
to impart to the resultant product highly desir-  
able and advantageous characteristics such as  
superior and lasting corrosion and scale resisting  
properties and luster or color, rendering the in-  
30 vention one of wide application and usefulness.

I have discovered that when organic salts of  
the desired coating and impregnating metals  
such as the formates, oxalates, acetates, etc. are  
35 packed about a foundation metal, such as iron  
and steel for example, and the whole heated in a  
closed receptacle to a temperature below the  
melting point of either metal, the salts decom-  
pose, liberating the metal constituent of the salt  
40 which in turn penetrates or enters the surface  
layer of the foundation metal and also forms a  
coating layer over the surface of such metal,  
these layers together constituting what may aptly  
be called a case comprised of substantially pure  
45 metal on the outside with a gradation inward of  
alloy decreasing in richness of coating and im-  
pregnating metal content from the surface to  
the interior of the foundation metal. By vary-  
ing the time and temperature of the treatment,  
50 the thickness or depth of the case may be varied.  
By way of example of the practice of the  
process, a mixture of 30 grams of nickel oxalate  
and one gram of iron chloride flux was packed  
about a low carbon steel article in a large tube  
55 closed at one end. This was inserted in a ver-  
tical electric furnace and the temperature raised

to approximately 1500° F. and held there for four  
hours. Nitrogen gas was introduced into the  
open end of the tube to displace the air. The ar-  
ticle, after this treatment and upon cooling,  
showed a nickelized case under the microscope  
5 with pure nickel on the outside and a gradual  
decline of the nickel content to the inside margin  
of the case. On etching a section of the article  
in dilute sulphuric acid, the case was plainly  
noticeable without magnification. It was from 10  
.005" to .025" in thickness. There was no sharp  
line between the case and core but a gradual  
change from the pure nickel on the outside to  
iron in the core, the inward portion of the case  
being a nickel iron alloy. Thus a case is formed 15  
which is firmly locked in the steel and is, in fact,  
an integral part of it. Crushing the impregnated  
article failed to show any cracking, separation, or  
other damage or impairment to the case.

If, in the above example, copper, chromium, 20  
or manganese oxalate were substituted for the  
nickel oxalate, the coating and impregnating  
case would be of copper, chromium, or man-  
ganese, and should it be desired to coat and im-  
pregnate the iron or steel with an alloy of two 25  
or more of these metals, a mixture of the organic  
salts of such metals would be used.

I have further discovered that in carrying out  
the process, the organic salts on decomposing  
generate inert and reducing gases such as carbon 30  
monoxide, carbon dioxide and hydrogen which  
protect the iron or steel from the air through-  
out the treatment, although under some condi-  
tions it may be found desirable to augment this  
protection by the addition of inert or reducing 35  
gases such as nitrogen or hydrogen from some  
outside source as in the above example. A quan-  
tity of some suitable fluxing material such as  
ferric-chloride or copper-chloride added to or  
mixed with the organic salt appears to expedite 40  
the penetration, although the process is entirely  
practical and workable without the use of an  
outside inert gas to augment the natural inert  
or reducing atmosphere generated and provided  
by the organic salts on heating. In fact, excellent 45  
results have been obtained by using merely the  
commercial organic salts and a flux and luting  
the receptacle to prevent oxidation. Metals other  
than iron or steel can be treated in a similar  
manner with similar results and organic salts of 50  
the desired impregnating metals other than the  
oxalates, formates, and acetates may be used,  
the chief requirement in this regard being that  
the selected salt be readily decomposable under  
heat to give off the desired coating and impre- 55

nating metal in atomic fineness and at the same time generate an inert or reducing gas which will protect the foundation metal from the air during the treatment.

5 In carrying out the process, the organic salt decomposes, liberating the impregnating metal in atomic fineness which is many times finer than it is possible to grind the metal. The impregnation of the metal in this form into the foundation metal proceeds with greater ease and rapidity and to a greater and more concentrated extent than under prior practices. The actual penetration is plainly shown by photomicrographs where it can be seen along and around 10 the grain boundaries of the foundation metal, and doubtless the impregnating metal also enters the grains themselves to form a solid solution which would not show in a photomicrograph because it would have the same grain structure as the 15 original ferrite. Along the grain boundaries the impregnating metal appears to be in a substantially pure state, while the grains themselves are of an alloy of the foundation and impregnating metals. Such alloy produced by my process may 20 be termed a cementation alloy as distinguished from an alloy produced by fusion.

I claim:

1. The process of coating and impregnating the 30 surface layer of one metal with another metal which consists in heating the first-named metal under non-oxidizing conditions in contact with an organic salt of a second-named metal at a temperature below the melting point of either of said metals, said organic salt being characterized 35 by the ability to yield inert and reducing gases such as carbon dioxide, carbon monoxide and hydrogen, when decomposed as a result of said heating.

2. The process of coating and impregnating the 40 surface layer of one metal with another metal which consists in heating the first-named metal under non-oxidizing conditions in contact with an organic salt of the second-named metal such as the oxalate, formate, or acetate thereof at a temperature below the melting point of either of said 45 metals, said organic salt being characterized by the ability to yield inert and reducing gases such as carbon dioxide, carbon monoxide and hydrogen, when decomposed as a result of said heating.

50 3. The process of coating and impregnating the surface layer of iron or steel with nickel which consists in heating the iron or steel under non-oxidizing conditions in contact with an organic salt of nickel such for example as nickel-formate, nickel-oxalate, or nickel-acetate to a temperature 55 at which the salt decomposes, said salt being characterized by the ability to yield inert and reducing gases such as carbon dioxide, carbon monoxide and hydrogen, when decomposed, liberating the nickel content thereof in the form of infinitesimally small particles which combine with the iron or steel by adhesion, intergranular penetration, and cementation.

60 4. The process of coating and impregnating the 65 surface layer of iron or steel with chromium which consists in heating the iron or steel under non-oxidizing conditions in contact with an organic salt of chromium such for example as chromium-formate, chromium-oxalate, or chromium-acetate to a temperature at which the salt decomposes, said salt being characterized by the 70 ability to yield inert and reducing gases such as carbon dioxide, carbon monoxide and hydrogen, when decomposed, liberating the chromium content thereof in the form of infinitesimally small

75 particles which combine with the iron or steel by adhesion, intergranular penetration, and cementation.

5 The process of coating and impregnating the surface layer of iron or steel with copper 5 which consists in heating the iron or steel under non-oxidizing conditions in contact with an organic salt of copper such for example as copper-formate, copper-oxalate, or copper-acetate to a 10 temperature at which the salt decomposes, said salt being characterized by the ability to yield inert and reducing gases such as carbon dioxide, carbon monoxide and hydrogen, when decomposed, liberating the copper content thereof in 15 the form of infinitesimally small particles which combine with the iron or steel by adhesion, intergranular penetration, and cementation.

6 A cementation compound for the treatment of iron or steel to provide the latter with a coating and impregnation in the form of a case of 20 non-oxidizing and corrosion resisting metal, consisting of an organic salt of the latter metal decomposable under heat, said salt being characterized by the ability to yield the metal constituent thereof in atomic fineness and inert and 25 reducing gases such as carbon dioxide, carbon monoxide and hydrogen.

7 A cementation compound for the treatment of iron or steel to provide the latter with a coating and impregnation in the form of a case of 30 non-oxidizing and corrosion resisting metal, consisting of an organic salt of the latter metal decomposable under heat, said salt being characterized by the ability to yield the metal constituent thereof in atomic fineness and an inert gas 35 which protects the iron or steel from the air during the treatment.

8 A cementation mixture for the treatment of iron or steel to provide the latter with a coating and impregnation in the form of a case of 40 non-oxidizing and corrosion resisting metal, consisting of an organic salt of the latter metal decomposable under heat, and a small quantity of fluxing material, said salt being characterized by the ability to yield the metal constituent thereof 45 in atomic fineness and an inert gas.

9 A cementation mixture for the treatment of iron or steel to provide the latter with a coating and impregnation in the form of a case comprised of an alloy of two or more non-oxidizing and corrosion resisting metals, which mixture consists 50 of organic salts of the latter metals decomposable under heat, said salts being characterized by the ability to yield the metal constituents thereof in atomic fineness and an inert gas.

10 A cementation mixture for the treatment of iron or steel to provide the latter with a coating and impregnation in the form of a case comprised of an alloy of two or more non-oxidizing and corrosion resisting metals, which mixture 60 consists of organic salts of the latter metals decomposable under heat, and a small quantity of fluxing material, said salts being characterized by the ability to yield the metal constituent thereof in atomic fineness and inert and reducing gases 65 such as carbon monoxide, carbon dioxide and hydrogen.

11 The process of coating and impregnating the surface layer of one metal with an alloy of 70 two or more metals which consists in heating the first-named metal under non-oxidizing conditions in contact with organic salts of the other metals at a temperature below the melting point of any 75 of said metals, said salts being characterized by

the ability to decompose under heat to yield inert and reducing gases.

12. The process of coating and impregnating the surface layer of one metal with another metal which consists in heating the first-named metal under non-oxidizing conditions in contact with a heat decomposable salt of the second-named metal, said salts being characterized by the ability to yield inert and reducing gases and to liberate the metallic constituent thereof in the form of infinitesimally small particles which combine with the first-named metal to form a case of substantially pure metal on the outside and a cementation alloy of the two metals on the inside.
13. The process of coating and impregnating
- the surface layer of iron or steel with a metal of the group consisting of chromium, nickel, copper and manganese which consists in heating the iron or steel under non-oxidizing conditions in contact with an organic salt of an acid of the group consisting of formic acid, oxalic acid and acetic acid of the desired metal of said first named group to a temperature at which the salt decomposes, said salts being characterized by the ability to yield inert and reducing gases when decomposed, liberating the metal content thereof in the form of infinitesimally small particles which combine with the iron or steel by adhesion, intergranular penetration, and cementation.

HARRY K. IHRIG.

15